# EUROPEAN PATENT SPECIFICATION

(11) **EP 1 478 515 B1**
(45) Date of publication and mention of the grant of the patent: **24.01.2007**
(21) Application number: 03742738.2
(22) Date of filing: 14.02.2003
(51) Int. Cl.: B41M 5/50

(54) **IMAGE RECEPTIVE MATERIAL COMPRISING CATIONICALLY CHARGED INORGANIC PARTICLES**
BILDAUFNAHMEMATERIAL,UMFASSEND KATIONISCH GELADENE ANORGANISCHE TEILCHEN
MATERIAU RECEPTEUR D'IMAGE COMPRENANT DES PARTICULES INORGANIQUES A CHARGE CATIONIQUE

(30) Priority: 19.02.2002 US 357863 P
(43) Date of publication of application: 24.11.2004
(73) Proprietor: 3M Innovative Properties Company, St. Paul, MN 55133-3427 (US)
(72) Inventor: GRAHAM, Paul, D., Saint Paul, MN 55133-3427 (US); SCHULZ, Mark, F., Saint Paul, MN 55133-3427 (US)
(74) Representative: Vossius & Partner
(86) International application number: PCT/US2003/004410
(87) International publication number: WO 2003/070477

(56) References cited:
- EP-A- 0 655 346
- EP-A- 1 008 457
- EP-A- 1 016 546

## Description

The present invention relates to ink receptive materials containing cationically charged inorganic particles and uses thereof. The present invention also relates to ink receptive materials containing inorganic particles.

To create a durable, high-quality image with an inkjet printer, careful attention must be given to the interactions between the ink and the imaging substrate. Proper control of such interactions often requires that a specially designed ink-receptive coating be applied to the film substrate of interest before the image is applied. Many inkjet inks are comprised of a relatively small amount of colorant materials that are dissolved or dispersed into a suitable vehicle. In many cases, the generation of high-quality images requires the ink-receptive coating to be designed so that it is able to absorb the ink vehicle before the ink is able to smear, run, or irregularly coalesce. For aqueous inkjet inks, suitable ink absorption is sometimes accomplished via the inclusion of water-swellable polymers into the ink-receptive coating.

Because the colorants used in aqueous inkjet inks may readily dissolve and/or redisperse in water and/or organic solvents, the creation of high-durability images requires that the coating is comprised of materials capable of forming durable bonds to the colorant, that is, mordants.

In applications where image durability is particularly important, it would be desirable to include high levels of mordants in image receptors to bond as many of the colorant molecules as possible. However, the incorporation of high levels of mordants in ink-receptive coatings may result in images having poor image quality. Poor image quality results because mordants are often not sufficiently water swellable to adequately control the final placement of the wet ink and to produce an image that is dry to the touch in a reasonable amount of time. Often, water-swellable materials are poor mordants.

As a second example, coatings comprised of the relatively high amount of the inorganic particles necessary to mordant certain colorants are often so brittle that they are impractical.

EP-A-0 655 346 discloses an ink jet recording sheet including a component of an ink receiving layer that consists mainly of non-spherical cationic colloidal silica, wherein the ink receiving layer is composed of a layer of coating formed by contour painting a surface of a substrate. In the sheet a, total quantity of charge of cations is specified, and a polyvinyl amine copolymer-containing substrate is used.

EP-A-1 008 457 relates to an ink jet recording sheet having on an ink-receiving support an image preserving layer comprising anionic colloidal silica and zinc oxide particulates with an average particle size of about 15 to 380 nm and having a 75 degree specular glossiness of at least about 25 % at the surface. Another ink jet recording sheet has on an ink-receiving support, in succession, an image preserving layer comprising anionic colloidal silica and zinc oxide particulates with an average particle size of about 15 to 380 nm and a fixing layer comprising cationic colloidal silica and cationic polymer electrolyte.

EP-A-1 016 546 describes an ink jet recording paper, comprising an ink-receiving layer and at least two colloidal silica layers applied successively onto a support, each of said colloidal silica layers comprising chain colloidal silica as a main ingredient, wherein at least the colloidal silica layer contacting the ink-receiving layer contains no binder and has a coverage of about 1 to 3 g/m², and the coverage of the other colloidal silica layer is about 1 to 6 g/m².

The present specification describes an ink receptor composition comprising or consisting essentially of, cationically charged inorganic particles. In another aspect, present specification describes an ink receptor composition comprising or consisting essentially of, cationically charged inorganic particles and an organic binder. In another aspect, present specification describes an ink receptor composition comprising or consisting essentially of, cationically charged inorganic particles and a mordant. In another aspect, present specification describes an ink receptor composition comprising or consisting essentially of, cationically charged inorganic particles, and organic binder, and a mordant.

The present invention provides an ink receptor composition comprising (a) alumina-coated silica particles prepared with an acetate stabilizing ion, or (b) zirconia particles prepared with an acetate stabilizing anion. Furthermore, the present invention relates to an ink receptor composition comprising a substrate having a surface; and a dried ink receptor composition as defined above on the surface. In addition, the present invention discloses a method of printing comprising the steps of applying ink to the above ink receptor medium using an inkjet printer.

Further embodiments of the present invention are described in the dependent claims.

An ink receptor composition of the invention comprises inorganic particles. Useful inorganic particles usually have a substantially positive charge on their surface (cationic) and are often supplied in acidic media. Useful inorganic particles include alumina-coated silica particles prepared with an acetate stabilizing ion (for example, TX11608, available from Ondeo Nalco Company, Chicago; IL) and zirconia particles prepared with an acetate stabilizing ion (that is, 00SS008 Zirconia sol, available from Ondeo Nalco Company, Chicago, IL). Useful inorganic particles are generally included into the ink receptor in an amount sufficient to form suitable interactions with the dyestuffs or colorant. The ink receptor compositions containing inorganic particles may contain about 1 to 100 percent dry weight percent inorganic particles, preferably from 30 to 100 percent dry weight percent inorganic particles, more preferably 50 to 100 percent dry weight percent inorganic particles and even more preferably from 60 to 95 percent dry weight percent inorganic particles.

The ink receptor compositions comprising inorganic particles may contain one or more mordants. A "mordant" as used herein is a material that forms a bond with dyestuffs or colorants in inks. A mordant is used to fix the ink dyestuffs so to provide increased durability to images, particularly water resistance. Useful mordants may include materials that are both water swellable and form a bond with dyestuffs or colorants in inks. Other useful mordants are those materials or compounds that contain cationic moieties, for example, quaternary amino groups. Desirably, the mordants do not interfere with the interactions between the inorganic particles and the dyestuffs or colorants in inks.

Useful mordants include, but are not limited to, FREETEX 685 (a polyquatemary amine, available from Noveon, Inc., Cleveland, OH), DYEFIX 3152 (an ammonium chloride-cyanoguanidine-formaldehyde copolymer, available from Bayer, Pittsburgh, PA), GLASCOL F207 (2-Propen-1-aminium, N,N-dimethyl-N-2-propenyl-, chloride, homopolymer, available from Ciba Specialty Chemicals), ECCOFIX FD-3 (a hydroxy-functional polyamide available from Eastern Color and Chemical, Providence, RI), SYNTRAN HX 31-65, SYNTRAN HX 31-44 (available from Interpolymer, Louisville, KY, both of which are copolymers wherein one of the monomers is selected from the group comprising alkyl methacrylate and alkyl acrylate, and one of the other monomers is selected from the group comprising quatemized dialkylaminoalkyl methacrylate and methyl, quaternized dialkylaminoalkyl acrylate).

The formation of suitable interactions with dyestuffs or colorants in inks may require the combination of inorganic particles and mordants.

The ink receptor compositions of the invention may contain up to about 80, up to about 70, up to about 60, up to about 50, up to about 40, up to about 30, up to about 20, or up to about 10 dry weight percent mordant. In other embodiments, the ink receptor compositions may contain 1 or greater, 5 or greater, 10 or greater, 20 or greater, 30 or greater, 40 or greater, or 50 or greater weight percent mordant on a dry basis. In other embodiments, the ink receptor compositions of the invention may contain from 40 to 90 dry weight percent mordant and any whole or fractional amount in between 40 and 90 dry weight percent. Water-swellable materials that do not bond to dyestuffs or colorants in inks are not used in inorganic particle ink receptor compositions of the invention are also useful. The ink receptor compositions of the invention may also contain one or more crosslinkers.

Optionally, a polymeric binder may be added to the ink receptor comprising inorganic particles to improve the adhesion between the particles arid a substrate. Useful polymeric binders provide adhesion to both the particles and the substrate and are compatible with the dispersion of inorganic particles. Poly(ethylene-co-vinyl acetate)-based polymers (such as those marketing by Air Products and Chemicals, Allentown, PA, by the AIRFLEX trade designation) and aromatic polyurethane-based polymers (such as those marketed by Zeneca Resins, Wilmington, MA, by the NeoRez trade designation) are examples. Particularly useful polymeric binders include AIRFLEX 400 (a poly(ethylene-co-vinyl acetate)-based emulsion, available from Air Products and Chemicals, Allentown, PA) and XR-9249 (an aromatic polyurethane-based polymeric emulsion, available from Zeneca Resins, Wilmington, MA). The polymeric binder may be generally included into the ink receptor in an amount sufficient to improve the adhesion between the inorganic particles and the substrate. The ink receptor compositions containing inorganic particles may include up to about 80 dry weight percent polymeric binder, preferably up to about 50 dry weight percent polymeric binder, more preferably from 5 to 40 dry weight percent polymeric binder, and even more preferably from 5 to 30 dry weight percent polymeric binder.

In another aspect, the invention comprises an ink receptor medium comprising a microembossed substrate comprising microembossed elements and an ink receptor comprising cationically charged inorganic particles on the microembossed surface. Preferably, the microembossed element is a cavity, post, or combination thereof. A "microembossed" surface has a topography wherein the average microembossed element pitch, that is, center to center distance between nearest elements is from 1 to 1,000 micrometers and may be any whole or fractional pitch in between 1 and 1,000 micrometers and the average peak to valley distances of individual elements is from 1 to 150 micrometers and any whole or fractional peak to valley distance between 1 and 150 micrometers. Preferably, if the microembossed elements are posts, the space between posts (pitch) is from 10 to 500 micrometers and any whole or fractional pitch between 10 and 500 micrometers, the posts have a height of from 10 to 100 micrometers, and diameters of not more than 100 micrometers and not less than 5 micrometers and any whole of fractional diameter between 5 and 100 micrometers.

In a particular embodiment, the microembossed surface comprises microembossed cavities. The volume of a cavity should preferably be at least 10 pL, and more preferably at least 30 pL. The volume of a cavity can range from 10 pL to 10,000 pL and may be any volume or volume range between 10 pL and 10,000 pL, and preferably from 60 pL to 8,000 pL and may be any volume or volume range between 60 pL and 8,000 pL. Other useful ranges of cavity volume include from 200 pL to 8,000 pL, and from 300 pL to 6,000 pL and may be any volume or range of volumes between 200 pL and 8,000 pL. Examples of topographies for cavities include conical cavities with angular, planar walls; truncated pyramid cavities with angular, planar walls; and cube-corner shaped cavities. Cavity depths can range from 15 to 150 micrometers and may be any depth or range of depths between 15 and 150 micrometers.

The microembossed pattern may be regular or random as described in U.S. Patent No. 6,386,699; U.S. Patent 6,649,249 also WO 00/73082; and U.S. Application Nos. 2003/0235678 and 2003/0235677, filed on June 25, 2002, respectively.

The substrate used in the ink receptor medium can generally be made from any polymer capable of being microembossed by methods known in the art. The substrate can be a solid film. The substrate can be transparent, translucent, or opaque, depending on desired usage. The substrate can be clear or tinted, depending on desired usage. The substrate can be optically transmissive, optically reflective, or optically retroreflective, depending on desired usage. The materials of the substrate may also depend upon the durability requirements of an image for a particular application, for example, an identification or security card. For such applications, poly(butylene terephthalate)-containing materials are preferred.

Nonlimiting examples of polymeric materials for use in such substrates include thermoplastics, such as those comprising polyolefins, poly(vinyl chloride), copolymers of ethylene with vinyl acetate or vinyl alcohol, polycarbonate, poly(butylene terephthalate), norbomene copolymers, fluorinated thermoplastics such as copolymers and terpolymers of hexafluoropropylene and surface modified versions thereof, poly(ethylene terephthalate), and copolymers thereof, polyurethanes, polyimides, polyamides, acrylics, plasticized polyvinyl alcohols, blends of polyvinylpyrrolidone and ethylene acrylic acid copolymer (Primacor^{™}, available from Dow Chemical Company) and filled versions of the above using fillers such as silicates, polymeric beads, aluminates, feldspar, talc, calcium carbonate, titanium dioxide, and the like. Also useful in the application are non-wovens, coextruded films, and laminated films made from the materials listed above.

Other useful substrates include substantially smooth substrates made from the materials listed above, and "beaded" substrates having exposed or partially exposed glass or polymeric beads or microbeads. Examples of exposed glass microbead substrates include those sold under the tradename CONFIRM Security Laminate, from 3M Company.

The ink receptor media of the invention may optionally have an adhesive layer on the major surface of the sheet opposite microembossed image surface that is also optionally but preferably protected by a release liner. After imaging, the ink receptor medium can be adhered to a horizontal or vertical, interior or exterior surface to warn, educate, entertain, advertise, etc.

The choice of adhesive and release liner depends on usage desired for the image graphic.

Pressure-sensitive adhesives can be any conventional pressure-sensitive adhesive that adheres to both the polymer sheet and to the surface of the item upon which the inkjet receptor medium having the permanent, precise image is destined to be placed. Pressure-sensitive adhesives are generally described in Satas, Ed., Handbook of Pressure Sensitive Adhesives, 2nd Ed. (Von Nostrand Reinhold 1989). Pressure-sensitive adhesives are commercially available from a number of sources. Particularly preferred are acrylate pressure-sensitive adhesives commercially available from 3M Company and generally described in U.S. Patent Nos. 5,141,790; 4,605,592; 5,045,386; and 5,229,207; and EPO Patent Publication No. EP 0 570 515 B1 (Steelman et al.).

Release liners are also well known and commercially available from a number of sources. Nonlimiting examples of release liners include silicone coated Kraft paper, silicone coated polyethylene coated paper, silicone coated or non-coated polymeric materials such as polyethylene or polypropylene, as well as the aforementioned base materials coated with polymeric release agents such as silicone urea, urethanes, and long chain alkyl acrylates, such as defined in U.S. Patent Nos. 3,957,724; 4,567,073; 4,313,988; 3,997,702; 4,614,667; 5,202,190; and 5,290,615; and those liners commercially available as Polyslik brand liners from Rexam Release of Oakbrook, IL, and EXHERE brand liners from P.H. Glatfelter Company of Spring Grove, PA.

In another embodiment, the ink receptor media of the invention further comprises a backing layer attached or laminated to the un-embossed surface of the microembossed substrate. The backing layer is used to provide the microembossed ink receptor media with thickness and rigidity, for example, for use as an identification card. As may be appreciated, the backing layer may be made from any material, with water proof and abrasion resistant materials being typical. Examples of useful materials include thermoplastics including those listed above and poly(ethylene terephthalate), poly(ethylene terephthalate glycol), polycarbonates, polyimides, cellulose acetate, poly(ethylene naphthalate), and polypropylenes, such as biaxially oriented polypropylene. The backing layer may be attached to the microembossed substrate by means known to those skilled in the art such as lamination, adhesive, or tape, and the like.

The microembossed surface can be made from any contacting technique such as casting, coating, or compressing techniques. More particularly, micro-embossing can be achieved by at least any of (1) casting a molten thermoplastic using a tool having a pattern, (2) coating of a fluid onto a tool having a pattern, solidifying the fluid, and removing the resulting micro-embossed solid, or (3) passing a thermoplastic film through a heated nip roll to compress against a tool having a pattern. Desired embossing topography can be formed in tools via any of a number of techniques well-known to those skilled in the art, selected depending in part upon the tool material and features of the desired topography. Illustrative techniques include etching (for example, via chemical etching, mechanical etching, or other ablative means such as laser ablation or reactive ion etching, etc.), photolithography, stereolithography, micromachining, knurling (for example, cutting knurling or acid enhanced knurling), scoring or cutting, etc.

Alternative methods of forming the micro-embossed image surface include thermoplastic extrusion, curable fluid coating methods, and embossing thermoplastic layers which can also be cured.

The ink receptors of the invention are typically formulated to receive an image comprising aqueous ink. The ink may be applied to the ink receptor by any means and in particular by means of an inkjet print head. Useful colorants in the inks include dye based colorants and pigment based colorants. Other examples of inks that may be useful for imaging ink receptors of the invention include non-aqueous inks, phase change inks, and radiation polymerizable inks.

### Examples

All of the amounts given are by weight unless otherwise stated. Unless otherwise stated, all of the components are available from Aldrich Chemical Co., Milwaukee, WI. Water used was de-ionized.
"TX-11608" is a trade designation for a 29 percent by weight dispersion of acetate-stabilized, alumina-coated colloidal silica, available from Ondeo Nalco Company, Chicago, IL.
"AIRFLEX^{®} 400 EMULSION" is a trade designation for a 52 percent by Weight latex emulsion, available from Air Products and Chemicals, Allentown, PA.
"DISPAL^{®} 18N4-80" is a trade designation for dispersible colloidal alumina powder, available from Sasol Ltd., Houston, TX.
"FREETEX^{®} 685" is a trade designation for a 50 percent by weight composition of a cationic polyamine available from Noveon, Inc., Cleveland, OH.
"HELOXY^{®} MODIFIER 48" is a trade designation for a polyfunctional epoxy crosslinker, available from Resolution Performance Products, Houston, TX.
"ECCOFIX FD-3" is a trade designation for a 30 percent by weight composition of a hydroxy-functional polyamide available from Eastern Color and Chemical, Providence, RI.
"SYNTRAN HX 31-65" is a trade designation for a 35 percent by weight composition of an acrylic copolymer, available from Interpolymer, Louisville, KY.

### Microembossed Film

The microembossed film was made by extruding a molten film into the roll nip formed by the top two rolls of a three roll calendering stack. The middle roll was a patterned metal roll. A portion of the surface of the metal patterned roll was engraved with an orthogonal set of grooves. Each of the grooves were spaced about 125 micrometers apart, about 75 micrometers deep, about 18 micrometers wide at their bottom and about 36 micrometers wide at their tops. The grooves were cut in a helical pattern around the roll such that the direction of each groove was oriented about 45 degrees from the roll axis. The temperature of the metal patterned roll was maintained at about 137.8 °C (280 °F) to about 160 °C (320 °F) using an oil bath. Water at 60 °C (140 °F) was circulated through the top roll and water at 90.56 °C (195 °F) was circulated through the bottom roll.

### Example 1

An ink receiving composition was prepared by mixing 10 parts TX-11608, 5 parts water, 1.67 parts n-propyl alcohol, and 1.45 parts AIRFLEX^{®} 400 EMULSION. The composition was mixed after each component was added. This ink receiving composition was applied with a #10 Mayer rod (nominal wet thickness = 0.023 mm) to the microembossed surface of a piece of microembossed film whose surface contained an array of square cavities that were about 70 micrometers deep and a microembossed element pitch of about 125 micrometers. The walls were about 18 micrometers thick at their top and about 36 micrometers at their bottom. The microembossed film was comprised of a 15:1 blend of CELANEX^{®} 1600A (a poly(butylene terephthalate), available from Ticona, Indianapolis, IN) and CELANEX^{®} 2020, color #EA3146K15 (a titanium dioxide containing color concentrate, available from Ticona) and was about 0.175 millimeters thick. The coated substrate was dried for five minutes in an oven at 70 °C (158 °F).

Several pieces of this the coated, microembossed film was attached with Scotch^{®} Brand Double Stick Tape (available from the 3M Company, St. Paul, MN) to a piece of about 0.550 millimeter thick PETG (poly(ethylene terephthalate glycol), available from the Eastman Chemical Co., Kingsport, TN) sheet.

This material was then printed onto the coated side using a Hewlett-Packard 845C inkjet printer that was specially modified to print thick materials and was equipped with a cartridge containing the same aqueous pigmented inkjet inks as in Cartridge Nos. C1892A, C1893A, C1894A, and/or C1895A, available from Hewlett-Packard, Palo Alto, CA. The resulting image exhibited high color density and excellent line sharpness with no bleed or feathering between colors.

Light finger pressure applied to the imaged surface of the film about two minutes after printing produce very little ink transfer. The imaged films were allowed to dry for about 24 hours before being placed into a standard laundry washing machine (Maytag, Model# LSE7804ACE) with 30 grams of AATCC 1993 Standard Reference Detergent (without optical brightener). The hot water and small load settings were used. The temperature of the hot water was about 43.33 °C (110 °F). After the imaged film went through the washing machine cycle, the image quality was virtually unchanged with very little bleed or feathering between colors.

### Example 2 (reference example)

The following compositions were prepared:
- Composition A:: Prepared by adding 6.25 parts DISPAL^{®} 18N4-80 to 18.75 parts water, then agitating vigorously in a high shear mixer for approximately 10 minutes. Then 40 parts water and 35 parts isopropanol were added with moderate mixing.
- Composition B:: Prepared by mixing 10 parts FREETEX^{®} 685 with 55 parts water and 35 parts isopropanol.
- Composition C:: Prepared by mixing 1 part HELOXY^{®} MODIFIER 48 with 39 parts isopropanol.
- Composition D:: Prepared by mixing 16.7 parts ECCOFIX FD-3 with 48.3 parts water and 35 parts isopropanol.
- Composition E:: Prepared by mixing 14.3 parts SYNTRAN HX31-65 with 42.9 parts isopropanol and 42.9 parts water.
- Composition F:: Prepared by mixing 70 parts of Composition A, 30 parts of Composition B, and 1.2 parts of Composition C.
- Composition G:: Prepared by mixing 70 parts of Composition A, 21 parts of Composition B, 9 parts of Composition D, and 1.2 parts of Composition C.
- Composition H:: Prepared by mixing 30 parts of Composition A, 70 parts of Composition E, and 2.8 parts of Composition C.

Compositions F, G, and H were each applied with a #10 Mayer rod (nominal wet thickness = 0.023 mm) to a microembossed surface of a piece of corona-treated microembossed film whose surface contained an array of square cavities that were about 70 micrometers deep and a microembossed element pitch of about 125 micrometers. The walls were about 18 micrometers thick at their top and about 36 micrometers at their bottom. The corona treatment was applied to the microembossed surface by passing a high frequency generator (120 volts, 50/60 Hertz, 0.35 amps, available from Electro Technic Products Inc., Chicago, IL) throughout the film surface. The microembossed film was comprised of a blend of 5 parts of Fina 3376 Polypropylene (available from Fina Oil and Chemical Co., Dallas, TX) and 1 part of P White 2% 10151005S (a titanium dioxide containing color concentrate in polypropylene available from Clariant, Charlotte, NC). The coated substrate was dried for about five minutes in an oven at 70 °C (158 °F).

This coated material was then printed onto the coated side using a Canon P-640L inkjet printer equipped with its standard ink cartridges. The printed film was placed into a convection oven for about 90 minutes at 70 °C (158 °F).

The color density of a printed black square was measured using a Gretag SPM 55 spectrophotometer. This portion of the film was submerged in room temperature water for about 80 minutes. The film was allowed to dry for about 24 hours and the black density was re-measured using the Gretag SPM 55 spectrophotometer. The table below shows a comparison of the black density before and after water submersion.

**Black Density**

| Film Coating | Before submersion | After submersion |
|---|---|---|
| Composition F | 0.946 | 0.908 |
| Composition G | 0.969 | 0.944 |
| Composition H | 0.930 | 0.926 |

## Claims

1. An ink receptor composition comprising (a) alumina-coated silica particles prepared with an acetate rotabilizing ion or (b) zirconia particles prepared with an acetate stabilizing ion.

2. The ink receptor composition of claim 1, further comprising a mordant.

3. The ink receptor composition of claim 1, wherein the cationically charged inorganic particles are present in an amount of from 30 to 100 percent dry weight, relative to the total weight of the ink receptor composition.

4. The ink receptor composition of claim 2, wherein the mordant is selected from the group consisting of polyquaternary amines, ammonium chloride-cyanoguanidine-formaldehyde copolymers, hydroxy-functional polyamides, (2-Propen-1-aminium, N,N-dimethyl-N-2-propenyl- chloride homopolymer), copolymers of alkyl methacrylate or alkyl acrylate with quaternized dialkylaminoalkyl methacrylate or methyl quaternized dialkylaminoalkyl acrylate, and combinations thereof.

5. The ink receptor composition of claim 2, wherein the mordant is present in an amount of up to 70 dry weight percent, relative to the total weight of the ink receptor composition.

6. The ink receptor composition of claim 1, further comprising a binder.

7. The ink receptor composition of claim 6, wherein the binder is a poly(ethylene-co-vinyl acetate)-based polymer, an aromatic polyurethane-based polymer; or combinations thereof.

8. An ink receptor medium comprising:
a substrate having a surface: and
a dried ink receptor composition of claim 1 on the surface.

9. The ink receptor medium of claim 8 wherein the surface of the substrate is substantially smooth, microembossed, or beaded.

10. The ink receptor medium of claim 9 wherein the microembossed surface comprinseavi6es, posts, or a combination of cavities and posts.

11. A method of printing comprising the steps of: applying ink to an ink receptor medium of claim 8 using an inkjet printer.

## Patentansprüche

1. Tintenaufnehmende Zusammensetzung, umfassend (a) Aluminiumoxid-beschichtete Siliciumdioxidteilchen, hergestellt mit einem Acetat-stabilisierenden Ion, oder (b) Zirkoniumoxid-Teilchen, hergestellt mit einem Acetat-stabilisierenden Ion.

2. Tintenaufnehmende Zusammensetzung nach Anspruch 1, ferner umfassend ein Mordent.

3. Tintenaufnehmende Zusammensetzung nach Anspruch 1, wobei die kationisch geladenen anorganischen Partikel in einer Menge von 30 bis 100 Prozent Trockengewicht relativ zum Gesamtgewicht der tintenaufnehmenden Zusammensetzung vorliegen.

4. Tintenaufnehmende Zusammensetzung nach Anspruch 2, wobei der Mordent ausgewählt ist aus der Gruppe, bestehend aus polyquartären Aminen, Ammoniumchlorid-Cyanoguanidin-Formaldehyd-Copolymeren, hydroxyfunktionellen Polyamiden, (2-Propen-1-aminium,N,N-dimethyl-N-2-propenylchloridhomopolymer), Copolymeren von Alkylmethacrylat oder Alkylacrylat mit quaternisiertem Dialkylaminoalkylmethacrylat oder Methyl-quaternisiertem Dialkylaminoalkylacrylat und Kombinationen davon.

5. Tintenaufnehmende Zusammensetzung nach Anspruch 2, wobei der Mordent in einer Menge von bis zu 70 Prozent Trockengewicht relativ zum Gesamtgewicht der tintenaufnehmenden Zusammensetzung vorliegt.

6. Tintenaufnehmende Zusammensetzung nach Anspruch 1, welche ferner ein Bindemittel umfasst.

7. Tintenaufnehmende Zusammensetzung nach Anspruch 6, wobei das Bindemittel ein Polymer auf Poly(ethylen-co-vinylacetat)-Basis; ein aromatisches Polymer auf Polyurethan-Basis oder Kombinationen daraus ist.

8. Tintenaufnehmendes Medium, umfassend:
ein Substrat mit einer Fläche und
eine getrocknete tintenaufnehmende Zusammensetzung nach Anspruch 1 auf der Fläche.

9. Tintenaufnehmendes Medium nach Anspruch 8, wobei die Fläche des Substrats im Wesentlichen glatt, mikrogeprägt oder mit Kugeln versehen ist.

10. Tintenaufnehmendes Medium nach Anspruch 9, wobei die mikrogeprägte Fläche Vertiefungen, Erhöhungen oder eine Kombination aus Vertiefungen und Erhöhungen umfasst.

11. Druckverfahren, umfassend den Schritt des Aufbringens von Tinte auf ein tintenaufnehmendes Medium nach Anspruch 8 unter Verwendung eines Tintenstrahldruckers.

## Revendications

1. Composition réceptrice d'encre comprenant (a) des particules de silice enrobées d'alumine préparées avec un ion stabilisant l'acétate ou (b) des particules de zircone préparées avec un ion stabilisant l'acétate.

2. Composition réceptrice d'encre selon la revendication 1, comprenant en outre un mordant.

3. Composition réceptrice d'encre selon la revendication 1, dans laquelle les particules minérales de charge cationique sont présentes, à raison de 30 à 100 pour cent en poids sec, par rapport au poids total de la composition réceptrice d'encre.

4. Composition réceptrice d'encre selon la revendication 2, dans laquelle le mordant est choisi dans le groupe constitué par les amines polyquaternaires, les copolymères chlorure d'ammonium-cyanoguanidine-formaldéhyde, les polyamides hydroxylés fonctionnels, (un homopolymère de 2-propén-1-aminium, de chlorure de N,N-diméthyl-N-2-propényle), les copolymères de méthacrylate d'alkyle ou d'acrylate d'alkyle avec du méthacrylate de dialkylaminoalkyle quaternisé ou de l'acrylate de méthyldialkylaminoalkyle quaternisé, et leurs combinaisons.

5. Composition réceptrice d'encre selon la revendication 2, dans laquelle le mordant est présent dans une proportion pouvant atteindre 70 pour cent en poids sec, par rapport au poids total de la composition réceptrice d'encre.

6. Composition réceptrice d'encre selon la revendication 1, comprenant en outre un liant.

7. Composition réceptrice d'encre selon la revendication 6, dans laquelle le liant est un polymère à base de poly(éthylène-co-acétate de vinyle), un polymère à base de polyuréthane aromatique, ou leurs combinaisons.

8. Support récepteur d'encre comprenant;
un substrat présentant une surface, et
sur la surface, une composition réceptrice d'encre séchée selon la revendication 1.

9. Support récepteur d'encre selon la revendication 8 dans lequel la surface du substrat est essentiellement lisse, microgaufrée ou perlée.

10. Support récepteur d'encre selon la revendication 9 dans lequel la surface microgaufrée comprend des creux, des bosses, ou une combinaison de creux et de bosses.

11. Procédé d'impression comprenant les étapes consistant à : appliquer une encre sur un support récepteur d'encre selon la revendication 8 au moyen d'une imprimante à jet d'encre.
